

## 1

3,413,074

## UNION DYEING AND PRINTING OF POLYESTER/CELLULOSE BLENDS

Albert Daaniel Lowande, Middlesex, and Alfred Louis Cate, Somerset, N.J., assignors to American Cyanamid Company, Stamford, Conn., a corporation of Maine  
No Drawing. Filed Aug. 31, 1967, Ser. No. 664,617  
4 Claims. (Cl. 8—21)

## ABSTRACT OF THE DISCLOSURE

Union dyeing or printing of polyester/cellulose blends is carried out by (1) applying to the fabric a padding solution or a printing paste comprising (a) a fiber-reactive dye characterized by the presence therein of a methyloated iminobispropionamide group attached to the dye by a defined type of bridging group, (b) a disperse dye having a Hot Press rating of 4-5 or 5, (c) an acid catalyst, such as ammonium chloride, and (d) water, and (2) drying the fabric at a temperature of 380-435° F. for from 5 seconds to 3 minutes. The dyed fabrics exhibit excellent fastness to washing as well as improved strength, brightness and fastness to light.

This invention relates to and has for its object the provision of an improved process for union dyeing or printing of polyester/cellulose blends and to a dye composition therefor.

More particularly, the invention relates to a process for union dyeing or printing of mixed or blended polyester and cellulose cloth or fabric. Thus, the fabric may be either blended at the yarn stage and subsequently woven into cloth or fabric, or not blended at the yarn stage but woven together into a cloth or fabric.

The process of the present invention makes it possible to produce (1) a solid or union shade or (2) contrast effects on polyester/cellulose fabrics. Thus, the process does not leave one of the mixed fibers undyed, but dyes both fibers simultaneously.

In accordance with the process of the invention, there is used in the pad bath or print paste, a dye reactive with cellulose under acid conditions having at least one iminobispropionamide radical, an acid catalyst, a disperse dye, water and, optionally, a thickener.

More than one of either type of dye, i.e., disperse or fiber-reactive, may be present in the pad bath or print paste. In accordance with the process the aqueous bath or paste is padded or printed onto the fabric, the fabric is dried and the dry fabric heated at a temperature above 380° F., but below the melting point of the polyester, until maximum fixation of the dyes to the respective fibers has taken place. Any unfixed dye is then removed.

The process of this invention differs from previous methods in providing an improved continuous simultaneous method of union dyeing and printing fabrics composed of both polyester and cellulose. Together the two types of dyes, disperse and reactive, are applied to the cloth, together they are dried and together at the same temperature they are fixed, excess or unfixed or unreacted dye being removed. Weakly acid conditions persist as long as there is moisture present. Alkalinity at any point in the process is avoided until union dyeing or printing is complete. Thereafter optionally the fabric is washed or soaped to remove excess unfixed dyes. During the removal of excess dye, mild alkali may be present although even here the use of neutral soaps or surface active agents is the usual practice.

Heretofore, when combinations of disperse and reactive dyes have been used for the union dyeing of polyester/cellulose blends, alkaline conditions have been used at that

## 2

part of the process where fixation of the reactive dye to cellulose takes place. The fiber-reactive dyes used in the alkaline process of the art differ in structure from the dyes used in the process of this invention. Such prior art dyes may have, for instance, a monochloro or dichlorotriazine moiety (Procion M or A dyes). Such dyes need alkaline conditions for fixation to cellulose. Also, heating in the presence of alkali has an adverse effect on the union shade. Furthermore, disperse dyes tend to be unstable in alkali at high temperature. Also, in the presence of alkali, fiber-reactive dyes can react with a reactive hydrogen if present in the disperse dye. Thus, fixation to the cellulose is substituted by fixation to the disperse dye with resultant loss of color value on the fabric.

The process of this invention is advantageous in that the dyes are not applied with urea. In the mill in the large quantities needed, urea has been found to yellow and dull light shades. It also causes corrosion problems with copper fittings in the drying and heating steps.

The fiber-reactive dyes of the invention are a new class of fiber-reactive dyes characterized by the presence therein of a methyloated iminobispropionamide group which is attached to the dye moiety through a particular type of "bridging group" which has an electron-withdrawing effect by virtue of which the dyes may be applied to cellulose in the presence of an acid catalyst. These new dyes are disclosed and claimed in a copending application of Frank F. Loffelman, Ser. No. 420,448, filed Dec. 22, 1964, now abandoned, and assigned to the assignee of the instant application. They conform to the formula:



where D is the residue of an organic dye moiety, Y is a bridging group selected from the group consisting of a covalent bond, sulfonyl, alkylsulfonyl, alkyleneoxy, alkyleneethio, carbonyl, alkyleneacarbonyl and alkylene, the alkylene radicals in Y having 1-2 carbon atoms; R is a member selected from hydrogen and alkyl carbons; R' is individually selected from the group consisting of hydrogen and the radical "—CH<sub>2</sub>OR" and n is a positive integer less than three.

As shown in the copending application, the radical "D" can be the moiety of any organic dye, the novel and characterizing feature of the new dyes being the



group. Numerous examples of the new class of dyes and their outstanding acid-fixing properties on cellulose are disclosed in the application Ser. No. 420,448.

The dyes fix over a wide range of temperatures, i.e., 300° F. to 435° F., which coincides with the range needed for the dyeing of polyesters, i.e., 380-430° F. They react well under slightly acid conditions which are also good for the Thermosol dyeing polyesters. They do not react with the fiber under alkaline conditions and thus are distinct from known reactive dyes used in conjunction with disperse dyes in dyeing polyester/cotton blends.

The disperse dyes used in the present invention should be chosen especially for their fastness to sublimation and



425° F., for 12 seconds, i.e., 6 seconds on each side, a similar result is obtained.

## EXAMPLE 2

## Continuous-union pad dyeing of polyester/cotton

A pad bath is prepared by mixing, diluting and dissolving with hot water in a pail, Dyes I, II and III (of Example 1) in amounts of 1.5 lb., 0.375 lb. and 4.5 lb. paste, respectively.

The solution of dye is added to a tank containing fifty gallons water at 110° F.; 9.0 lb. solution of natural gums and 3.0 lb. ammonium chloride are added. The whole is diluted to 75 gal. with water.

Five hundred yards of 50/50 polyester/cotton are padded with this solution at a rate of 70 yards per minute, skyed, predried by infrared and dried by four hot roll cylinders at 180°, 250°, 250° and 350° F., respectively. The fabric is heat-treated for nine seconds by contact with ten rolls at 400-435° F.

Following this, the yardage is rinsed, soaped at 180° F., in water containing 1 lb./100 gallons of an anionic detergent, sodium N-methyl-N-oleyl taurate, rinsed and dried. The union-dyed fabric obtained is a medium pink shade. It is uniformly dyed with no shade differences from face to back or sides to center.

The procedure is the same as for Example 3.

A full blue union shade is obtained of excellent fastness to washing.

## EXAMPLE 6

## Union printing of polyester/cotton

A print paste is made by mixing the dyes listed in Table I in the amounts shown with 75 grams of a sodium alginate emulsion prepared by homogenizing:

10 20 grams of sodium alginate granules stirred to a paste with 545 ml. water;  
10 grams of a surfactant disodium N-octadecylsulfosuccinate, and  
445 grams of a petroleum solvent distilling between 321 and 388° F.

15 Ammonium chloride solution in the amount shown in the table is added. Sufficient water is added to bring the printing paste to 100 grams.

20 The paste is printed on 65/35 polyester/cotton poplin fabric. It is dried and subjected to heat at 400° F. for 90 seconds. The print is rinsed in cold water, soaped in 2 g./liter neutral soap solution at the boil for 5 minutes rinsed in hot water, squeezed and pressed dry. A full range of uniform excellent medium shades are obtained on the fabric as shown in the table.

TABLE I.—PRINT FORMULATIONS IN GRAMS OF DYE PER 100 GRAMS PRINTING PASTE

|        | Fiber reactive dye |      |      | Disperse dye |       |      | 10% NH <sub>4</sub> Cl solution in ml. | Union shade on polyester/cotton |
|--------|--------------------|------|------|--------------|-------|------|----------------------------------------|---------------------------------|
|        | I                  | II   | III  | III          | V     | VI   |                                        |                                 |
| 1----- | 1.00               | 1.00 | 0.00 | 2.15         | 0.012 | 0.00 | 0.5                                    | Red.                            |
| 2----- | 0.75               | 1.00 | 0.00 | 1.50         | 0.125 | 0.00 | 0.5                                    | Scarlet.                        |
| 3----- | 1.00               | 6.00 | 0.00 | 2.20         | 1.00  | 0.00 | 0.5                                    | Orange.                         |
| 4----- | 0.00               | 2.00 | 0.00 | 0.00         | 0.50  | 0.00 | 0.5                                    | Yellow.                         |
| 5----- | 0.00               | 2.00 | 2.00 | 0.00         | 0.35  | 0.00 | 0.5                                    | Green.                          |
| 6----- | 0.00               | 0.00 | 2.00 | 0.00         | 0.00  | 0.00 | 0.5                                    | Turquoise.                      |
| 7----- | 0.25               | 0.00 | 1.50 | 0.25         | 0.00  | 0.00 | 0.5                                    | Blue.                           |
| 8----- | 1.00               | 3.00 | 1.50 | 1.50         | 0.35  | 0.75 | 0.5                                    | Gray.                           |

## EXAMPLE 3

## Red union dyeing of polyester/cotton fabric

A pad bath is made up having a concentration per liter of

40 Grams  
Dye I of Example 1 ----- 20  
Dye III of Example 1 ----- 40  
Ammonium chloride ----- 0.5  
Sodium alginate ----- 2

45 The bath is adjusted to pH 6.8 with dilute hydrochloric acid. A 65/35 polyester/cotton blended fabric is padded, dried and cured at 410° F. for 90 seconds. It is then rinsed and soaped.

50 A full blue-red union shade is obtained of excellent fastness to washing.

## EXAMPLE 4

## Yellow union dyeing of polyester/cotton fabrics

55 A pad bath is prepared as in Example 3, except that instead of Dyes I and II of Example 1, Dye II of Example 1 and a nitro dye of the formula:



60 are used in amounts of 20 g. powder and 30 g. double paste, respectively. Otherwise, the procedure of Example 3 is followed.

65 A full green-yellow union shade is obtained of excellent fastness to washing.

## EXAMPLE 5

## Blue union dyeings of polyester/cotton fabric

70 A pad bath is prepared, containing per liter

Grams  
Dye IV of Example 6 ----- 16  
Dye I of Example 1 ----- 0.7  
Dye III of Example 1 ----- 1.0

55 The prints obtained have good fastness to AATCC Tests Wash No. 2A, Acid Perspiration, Alkaline Perspiration, Dry Cropping and Dry Cleaning.

The dyes of Table I are identified as follows:

Dyes I and II are Dyes I and II of Example 1.

Dye IV is a copper phthalocyanine dye of the structure:



50 Dye III is Dye III of Example 1.

Dye V is:



55 Dye VI is a substituted quinizarine.

We claim:

1. Process for union dyeing or printing of fabric composed of cellulose and polyester which comprises

(1) applying to the fabric a padding solution or a printing paste comprised of:

(a) a fiber-reactive dye of the formula



- wherein D is the residue of an organic dye moiety, Y is a bridging group selected from the group consisting of a covalent bond, sulfonyl, alkylenesulfonyl, alkyleneoxy, alkyleneethio, carbonyl, alklenecarbonyl and alkylene, the alkylene radicals in Y having 1-2 carbon atoms; R is a member selected from hydrogen and alkyl of 1-4 carbons; R' is individually selected from the group consisting of hydrogen and the radical "—CH<sub>2</sub>OR" and n is a positive integer less than 3; 10
- (b) a disperse dye having a rating of 4-5 or 5 in Hot Pressing as shown in the Colour Index, 2nd edition, vol. I, page 1655-1742;
- (c) an acid catalyst, and 15
- (d) water, and
- (2) drying the fabric at a temperature of 380-435° F. for from 5 seconds to 3 minutes.

2. A process according to claim 1 in which the acid catalyst is ammonium chloride present in an amount of 20 from 0.25 to 4.0 g. per liter.

3. A dye composition comprising:
- (a) a fiber-reactive dye of the formula



wherein D is the residue of an organic dye moiety,

Y is a bridging group selected from the group consisting of a covalent bond, sulfonyl, alkylenesulfonyl, alkyleneoxy, alkyleneethio, carbonyl, alklenecarbonyl and alkylene, the alkylene radicals in Y having 1-2 carbon atoms; R is a member selected from hydrogen and alkyl of 1-4 carbons; R' is individually selected from the group consisting of hydrogen and the radical "—CH<sub>2</sub>OR" and n is a positive integer less than three;

- (b) a disperse dye having a rating of 4-5 or 5 in Hot Pressing as shown in the Colour Index, 2nd edition, vol. I, page 1655-1742;
- (c) an acid catalyst; and
- (d) water.

15 4. A dye composition according to claim 3, in which the acid catalyst is ammonium chloride present in an amount of from 0.25 to 4.0 g. per liter.

#### References Cited

##### UNITED STATES PATENTS

2,346,013 4/1944 Dickey ----- 260—199 XR  
3,066,005 11/1962 Wedemeyer ----- 8—17 XR

##### FOREIGN PATENTS

25 805,562 12/1958 Great Britain.

##### OTHER REFERENCES

Frick et al.: American Dyestuff Reporter, vol. 51, No. 23, pp. 45-48.

30 NORMAN G. TORCHIN, Primary Examiner.

D. LEVY, Assistant Examiner.